

## UNITED STATES PATENT OFFICE

2,214,331

## ELECTRODEPOSITION OF ZINC

Richard O. Hull, Lakewood, Ohio, assignor to E. I.  
du Pont de Nemours & Company, Wilmington,  
Del., a corporation of Delaware

No Drawing. Application April 27, 1937,  
Serial No. 139,203

6 Claims. (Cl. 204—18)

This invention relates to the electrodeposition of zinc, and is particularly directed to the use of zinc anodes which contain small amounts of calcium.

5 In processes for the electrodeposition of zinc it is customary to maintain the zinc content of the zinc plating baths by the use of zinc anodes, but considerable difficulty is experienced by reason of the fact that the anode efficiency is greater than the cathode efficiency. In other words, 10 the zinc metal of the anode is dissolved in the bath more rapidly than zinc metal is deposited from the bath onto objects being plated. As a result of the rapid solution of the anode the 15 bath soon contains excessive amounts of zinc compounds.

For the best results it is desirable that a zinc plating bath remain as near as possible to a definite formula, and changes in bath composition 20 resulting from the rapid solution of zinc anodes cause considerable difficulty. In the recently developed processes for the electrodeposition of bright zinc deposits it is particularly important that the bath composition be held rigidly within limits if the best possible results are 25 consistently to be obtained.

In addition to the difficulties arising from the rapid solution of zinc anodes in zinc plating baths, further difficulties result from the fact 30 that the anodes do not dissolve evenly and from the fact that a black sludge is formed which floats in the bath and on the surface of the bath. The presence of black sludge is particularly disadvantageous in processes for the deposition 35 of bright zinc from cyanide baths since this black sludge interferes with the production of a smooth and bright plate.

When a zinc plating bath has such an amount 40 of zinc dissolved therein that it becomes necessary to correct the bath composition, this can be done by removing some of the zinc. Or, as is more customarily the practice, the excess of zinc compounds may be diminished by discarding a portion of the solution and correcting the composition 45 of the remaining solution by the addition of bath constituents other than zinc compounds. It will of course be apparent that such procedures are uneconomical and time-consuming.

50 It has been proposed to compensate for the high anode efficiency of zinc anodes in cyanide baths by replacing some of them with insoluble iron or steel anodes. This expedient results in a diminution of the amount of zinc dissolved per

unit of electrical current passed into the bath, and in effect reduces the anode efficiency.

Unfortunately this type of procedure is not entirely satisfactory because when the bath is standing idle the iron or steel anodes accelerate the rate of corrosion of the zinc anodes, thus causing the zinc to dissolve rapidly and unevenly during periods when the bath is not in operation. It is, moreover, generally accepted that insoluble anodes cause destructive oxidation of cyanide during electrolysis. Such oxidation is considered to destroy the valuable cyanides and to produce deleterious carbonates.

5 It has also been proposed to use zinc-aluminum alloy anodes. By such use of aluminum in a zinc anode the anode efficiency is slightly decreased since zinc-aluminum alloys are slightly less soluble than pure zinc metal. This proposed use of zinc-aluminum alloy anodes was 10 primarily suggested for acid-zinc plating baths 15 and has been found most useful in this relation.

Unfortunately the use of aluminum in zinc anodes does not solve the problem of maintaining zinc plating baths at a constant composition. The effect of adding aluminum is too small to 20 secure a balance of anode and cathode efficiencies. This is particularly true when the anodes are used in cyanide baths, perhaps because the 25 aluminum is alkali soluble.

I have found that the difficulties heretofore 30 experienced in the art may largely be overcome by the addition of moderately small amounts of calcium to zinc anodes. By selecting a proper amount of calcium, anodes having an efficiency 35 corresponding closely to the cathode efficiency of the baths in which they are to be used may readily be produced. By the use of such anodes it is possible to maintain the balance of bath constituents for a much longer period than has heretofore been practicable, particularly with 40 cyanide baths.

The use of the zinc-calcium anodes of my invention is particularly advantageous in conjunction 45 with cyanide-zinc plating baths for the deposition of bright zinc deposits since by the use of the anodes of my invention it is possible to hold the bath composition within rigid limits with a minimum of effort and cost.

The zinc-calcium alloy anodes of my invention 50 are further characterized by the fact that they dissolve uniformly in zinc plating baths and produce a minimum amount of black sludge. Particularly when relatively large amounts of calcium, say in the range around 0.5%, is used, the amount of black sludge is markedly de- 55

creased. In any event the presence of calcium in the anode causes any black sludge which does form to settle directly to the bottom of the bath and the disadvantage heretofore encountered of 5 the black sludge floating in the bath and on the surface of the bath is obviated. The action of calcium in promoting even corrosion and in preventing deleterious black sludge formations makes the zinc-calcium alloy anodes of my invention 10 particularly valuable for use in cyanide-zinc plating baths for the production of bright smooth deposits.

The action of calcium in the zinc-calcium alloys of my invention is entirely different from 15 the action of metals such as aluminum. Aluminum, for instance, is itself soluble in both acid and cyanide-zinc plating baths and zinc alloys containing it are likewise soluble, the they dissolve slightly less rapidly than pure zinc.

20 Calcium on the contrary is not soluble in cyanide-zinc plating baths. The calcium in the zinc-calcium anodes of my invention apparently causes the formation of a film of alkali-insoluble calcium compound on the surface of 25 anodes which are in use. This film polarizes the anodes, in a measure resisting the passage of current between the anode and the bath. The effect of the calcium is directly proportional to the amount present, and by the use of a suitably 30 large amount of calcium, zinc-calcium alloys of almost any desired efficiency can be made.

Electrolytic zinc anodes for use in cyanide-zinc plating baths normally have an anode efficiency of 100 to 105%, while the normal cathode 35 efficiency in similar baths is around 80 to 95%. The anode efficiency of such electrolytic zinc anodes may be reduced to fall within the range of cathode efficiencies by the addition of calcium to the zinc metal, for instance, 1% of calcium 40 being sufficient under one set of conditions to give an electrolytic zinc-calcium alloy anode having an anode efficiency of 85%. It is of course particularly desirable to be able to reduce the anode efficiency of electrolytic zinc anodes 45 because the high purity of this type of anode renders it desirable for bright zinc processes.

Many zinc anodes however are not made from electrolytic zinc but are made of somewhat less pure zinc obtained by distillation methods. 50 These anodes are much used for zinc plating, and they have found considerable application in the plating of bright zinc from cyanide-zinc plating baths. These less pure anodes dissolve somewhat more slowly than do the electrolytic anodes, 55 the usual anode efficiency being around 100% for commercial grade zinc anodes.

Considerably smaller amounts of calcium are sufficient to reduce the anode efficiency of zinc anodes to the required amount when commercial 60 zinc from distillation processes is used. For instance 0.6% of calcium was sufficient to give a zinc-calcium anode having an efficiency of 85% when the zinc was of a commercial grade obtained by distillation.

65 The use of calcium is particularly advantageous with the use of anodes which are less pure than the electrolytic zinc because the calcium tends to reduce the amount of black sludge 70 formed and further causes this sludge to drop to the bottom of the tank where it cannot interfere with the bright plates. As a result, it is entirely feasible to produce brilliant zinc plates from cyanide-zinc plating baths using commercial grades of zinc obtained by distillation 75

if calcium is incorporated in the metal according to the teachings of my invention.

It will readily be understood that various other metals may be included in the zinc anodes in conjunction with calcium in accordance with 5 the practices already known in the art. I may for instance use calcium jointly with aluminum or mercury, or I may use all three to obtain their joint effects.

It will further be apparent that since the impurities present in commercial grades of zinc co-operate with calcium to produce anodes of low efficiency it may conceivably be advantageous in some circumstances to add such impurities jointly with calcium to zinc metal which, by 15 reason of its higher purity, dissolves too rapidly and would require an excessive amount of calcium to obtain the desired anode efficiency. This is particularly true because of the present 20 high price of calcium metal.

In order that my invention may be better understood, the following examples are given:

#### Example I

Molten zinc obtained in a zinc distillation process was transferred in the molten state to a gas-fired graphite crucible and the temperature raised from about 450° C. up to a temperature of about 600° C. Five-tenths per cent of calcium was then added to the zinc by introducing calcium turnings into the molten zinc and maintaining them below the surface until they were dissolved in the zinc. After the calcium was alloyed with the zinc, the mixture was further heated and the alloy was then cast into a form 30 suitable for use as anodes.

The zinc used was of commercial grade frequently employed for the manufacture of zinc anodes. The zinc contained about 0.07% of cadmium and 0.005% of iron. It also contained 40 0.10% of lead and the cast anodes, accordingly, contained these impurities in addition to the added calcium. For testing the anodes, a cyanide-zinc plating bath of the type recently developed for the deposition of brilliant zinc was made 45 up as follows:

|                             | Grams per liter |
|-----------------------------|-----------------|
| Zinc cyanide ( $Zn(CN)_2$ ) | 60              |
| Sodium cyanide ( $NaCN$ )   | 52.5            |
| Sodium hydroxide ( $NaOH$ ) | 78              |
| Molybdcic acid ( $MoO_3$ )  | 50              |
|                             | 7.5             |

Using the above bath and the zinc-calcium alloy anodes above produced, excellent deposits were obtained. The anodes dissolved fairly evenly and without the formation of deleterious black sludge. The small amount of sludge which formed sank to the bottom of the bath and did not interfere with the plating operation.

The anode efficiency was determined and it was found that the anodes made as above described and containing 0.5% of calcium had an efficiency of about 85% in the above bath.

#### Example II

A zinc-calcium alloy anode was made up according to the procedure described in the above Example I, but using 0.6% of calcium. The zinc used was somewhat purer than that of the above example, containing only 0.05% of lead. In making the alloy 0.05% of lead was added to decrease the solubility of the anodes.

After the alloy was cast into a suitable form, the anodes were tested in a bath such as that shown in Example I and were found to have an anode efficiency of about 84%.

Since the presence of lead is so undesirable in baths for the deposition of bright zinc it does not at first appear practical to add this impurity to the zinc metal. The calcium, however, is so efficacious in preventing the deleterious action of lead and other such impurities that it is satisfactory to gain the benefits which may be had by using lead and saving on the more expensive calcium.

- 10 As indicated above, the calcium probably acts by forming an alkali-insoluble calcium hydrate or cyanide film which surrounds the particles of lead and drags them to the bottom of the bath where they can do no harm. It will be observed, 15 of course, that there must be sufficient calcium present since otherwise the lead would be free to exercise a deleterious influence.

*Example III*

- 20 A zinc-calcium alloy anode was made by using electrolytic zinc and 1.07% of calcium. The alloy was made following the procedure used in the above Example I, the electrolytic zinc being melted directly in the graphite crucible. The zinc-calcium alloy anodes so produced were tested in a bright zinc bath such as that shown above in Example I and it was found that the anode efficiency was about 82%.

While I have shown specific conditions in the foregoing for the production of zinc-calcium alloy anodes, it will be understood that these may be made in various ways according to known metallurgical practices. It is to be observed, however, that after the calcium is added to the zinc, the mixture should be heated to a temperature not substantially lower than about 800° C. In making up one set of electrolytic zinc anodes this precaution was not observed, the metal being poured at a temperature somewhere slightly above 600° C. and the alloy anodes so produced had an efficiency only slightly lower than that of electrolytic zinc itself. The specific temperature required to effect the required change in alloy properties can readily be determined in each specific instance by a few simple trials. The electrolytic zinc alloy anodes mentioned were remelted and heated to a temperature of 800° C. and it was then found that the calcium exercised its usual profound effect upon the anode efficiency.

From the foregoing it will be evident that widely varying amounts of calcium may be used depending upon the effect desired and upon the character of the zinc which it is desired to modify. By the use of suitable amounts of calcium it is entirely possible to adjust the anode efficiency to correspond to the cathode efficiency of substantially any commercial cyanide-zinc electroplating bath and it is principally in this connection that the invention will be found valuable. It will be understood, however, that the beneficial effects of calcium may be obtained by the use of small amounts of calcium which will prevent the deleterious influence of metal impurities in the anode even without obtaining a very great reduction in

the anode efficiency. Very small amounts of calcium may therefore be used to advantage.

Larger amounts of calcium may of course be used, tho it will be understood that it will not be commercial to use large amounts. In general, of course, the upper limit on the amount of calcium used is determined by the cathode efficiency of the baths in which the anodes are to be employed and by economic considerations.

While, as above indicated, widely varying amounts of calcium may be used, it will generally be found desirable to use from about 0.05% to about 5.0% of calcium. More specifically, it will usually be found that the desired anode efficiency and character can be obtained using from about 0.25% to 1.5% of calcium with electrolytic zinc or about 0.25% to 1.0% of calcium with commercial zinc such as that shown in Examples I and II and obtained by distillation processes.

The zinc-calcium alloy anodes of my invention have been particularly discussed above in conjunction with their use in a particular cyanide-zinc plating bath, but it will be understood that the type of anodes of my invention may advantageously be employed in conjunction with various other such cyanide-zinc electroplating baths.

I claim:

1. In a process for the electrodeposition of zinc from a cyanide-zinc plating bath, the step comprising employing a zinc anode which has an efficiency substantially corresponding to the cathode efficiency of the bath, the anode efficiency being decreased by the inclusion in the anode of a small amount of calcium.

2. In a process for the electrodeposition of zinc from a cyanide-zinc plating bath, the step comprising employing a zinc anode which contains from about 0.05 to 5.0 per cent of calcium the calcium effecting a diminution of the anode efficiency.

3. In a process for the electrodeposition of zinc from a cyanide-zinc plating bath, the step comprising employing a zinc anode which contains lead and a small amount of calcium, the calcium effecting a diminution of the anode efficiency.

4. In a process for the electrodeposition of zinc from a cyanide-zinc plating bath, the step comprising employing an electrolytic zinc anode which contains a small amount of calcium, the calcium effecting a diminution of the anode efficiency.

5. In a process for the electrodeposition of zinc from a cyanide-zinc plating bath, the step comprising employing a zinc anode which contains lead as an impurity and which contains from about 0.25 to 1.0 per cent of calcium, the calcium effecting a diminution of the anode efficiency.

6. In a process for the electrodeposition of zinc from a cyanide-zinc plating bath, the step comprising employing an electrolytic zinc anode which contains from about 0.25 to 1.5 per cent of calcium, the calcium effecting a diminution of the anode efficiency.

RICHARD O. HULL.